

UNITED STATES PATENT OFFICE

2.038.081

# **WATER-INSOLUBLE AZO-DYE STUFFS AND FIBER DYED THEREWITH**

**Leopold Laska, Offenbach-on-the-Main, Arthur Zitscher, Kronberg-in-the-Taunus, and Wilhelm Seidenfaden, Offenbach-on-the-Main, Germany, assignors to General Aniline Works, Inc., New York, N. Y., a corporation of Delaware**

**No Drawing. Application July 3, 1935, Serial No.  
29,730. In Germany July 16, 1934**

**10 Claims. (Cl. 260—95)**

The present invention relates to water-insoluble azo-dyestuffs and to fiber dyed therewith; more particularly it relates to dyestuffs corresponding to the following general formula



wherein X stands for hydrogen, halogen or an alkoxy group.

15 We have found that valuable azo-dyestuffs insoluble in water are obtained by coupling the diazo-compound of 4-amino-3,4'-dinitrodiphenylamine with an arylide of 2,3-hydroxy-naphthoic acid in substance, on the fiber or on a substratum  
20 adapted for the production of lakes. In this manner black-currant to black dyeings of remarkable fastness properties, particularly of very good fastness to light, are obtained.

The new dyestuffs may be used for the production on the fiber of dyeings and printings, as well as for the preparation of pigments.

The dyestuffs may furthermore be used for the production on the fiber of mixed shades with other dyestuffs derived from the group of the 30 2,3-hydroxynaphthoic acid arylides, for instance, with those from the diazo-compounds of 4-aminodiphenylamines; this is of particular technical importance, since in this manner the tints of those dyestuffs may be darkened as required.

35      Similar combinations have been described in U. S. Patents Nos. 1,919,589 and 1,921,362. According to the process of the present invention there are obtained black-currant and black dyeings of great commercial value, whereas according 40 to the processes described in the said patents there are obtained only garnet to blue or violet shades which are, moreover, less fast to light than the combinations obtainable by the process of the present invention. Moreover, the combinations 45 of the present process, when used for dyeing piece goods, have a greater tinctorial strength than those obtainable according to U. S. Patent No. 1,921,362.

50 The following examples serve to illustrate the invention, but they are not intended to limit it thereto.

(1) 4 grams of 1-(2',3'-hydroxynaphthoyl)-aminonaphthalene are dissolved by boiling with 55 10 cc. of Turkey red oil, 12 cc. of caustic soda.

solution of 34° Bé. and 100 cc. of hot soft water, 100 cc. of cold soft water and 4 cc. of formaldehyde of 33 per cent strength are then added to the solution. The formaldehyde is allowed to act for 5 minutes whereupon the grounding liquor is made up to 1000 cc. 5

In the bath thus prepared, the yarn, pre-treated in the usual manner, is impregnated at 30° C. for 30 minutes. After hydro-extracting, the impregnated yarn is developed in a bath containing per liter 4.42 grams of 3,4'-dinitrodi-phenylamine-4-diazonium chloride of net content of 62 per cent calculated upon the base and 1.8 cc. of acetic acid of 50 per cent strength. 10

The material is thoroughly rinsed cold and hot and soaped at boiling temperature. A greenish black shade of good fastness to light is obtained. The dyestuff is characterized by the following formula:



In the same manner the following shades are obtained with the 2,3-hydroxynaphthoyl-compound of

|                                                                         |                 |    |
|-------------------------------------------------------------------------|-----------------|----|
| 1-amino-2-methoxybenzene                                                | Greenish black, | 35 |
| 1-amino-2-methylbenzene                                                 | Greenish black, |    |
| 1-amino-4-methoxy- 2 -methylbenzene                                     | Violet black,   |    |
| 1-amino-2,4-dimethoxy- 5 -chlorobenzene                                 | Violet black,   | 40 |
| 1-amino-2,5-dimethoxybenzene                                            | Black-currant,  |    |
| 1 - amino - 4 - methoxynaphthalene                                      | Black-currant,  |    |
| 1-amino-2,4-dimethoxybenzene                                            | Violet-black,   | 45 |
| 1-amino-2,5-dimethoxy-4 -chlorobenzene                                  | Black-currant,  |    |
| and with                                                                |                 |    |
| 6' -bromo - 2',3' - hydroxynaphthoyl-(1-amino - 2,4 - dimethoxybenzene) | Violet black,   | 50 |
| 6'-methoxy-2',3'-hydroxynaphthoyl-(1 - amino - 2 - methoxybenzene)      | Greenish black. | 55 |

(2) PRINTING ON GOODS PREPARED WITH 1-(2',3'-HYDROXY-NAPHTHOYL)-AMINO-2-METHYLBENZENE  
*Grounding liquor*

5 15 grams of 1-(2',3'-hydroxynaphthoyl)-amino-  
 2-methylbenzene are made into a paste  
 with  
 15 cc. of Turkey red oil and  
 22.5 cc. of caustic soda solution of 34° Bé. and  
 10 the paste is dissolved in and made up  
 with hot water to

1 liter.

The goods are impregnated on a foulard at 50° C.  
 15 and dried.

*Printing paste*

17 grams of the diazonium chloride from 4-  
 amino-3,4'-dinitro-diphenylamine,  
 20 grams of acetic acid of 50 per cent strength,  
 20 453 grams of water,  
 10 grams of the condensation product of oleyl  
 alcohol and ethylene oxide  
 500 grams of neutral starch tragacanth thick-  
 ening

25 1000 grams.

After printing, the material is dried, then  
 treated with hot sodium carbonate solution (con-  
 taining 1 to 2 grams of calcined sodium carbo-  
 nate per liter, rinsed and soaped.

30 A deep greenish black shade is obtained.

(3) PIECE DYEING

Crude desized cotton piece goods are impreg-  
 nated at 80° C. on a foulard with the following  
 35 solution:

12 grams of 1-(2',3'-hydroxynaphthoyl)-amino-  
 2-methoxy-benzene are made into a  
 paste with  
 40 12 cc. of Turkey red oil and  
 18 cc. of caustic soda solution of 34° Bé. The  
 paste is dissolved in hot water and  
 made up to

45 1 liter.

Then the goods are dried.

*Developing bath*

10 grams of the diazonium chloride from 4-  
 amino-3,4'-dinitro-diphenylamine are  
 50 dissolved in  
 10 grams of acetic acid of 50 per cent strength  
 and  
 300 cc. of hot water and made up to

55 1 liter.

The impregnated and dried goods are passed on  
 a foulard at 50° C. through this developing solu-  
 tion and then passed through a steam chest  
 60 wherein they are steamed for about half a min-  
 ute. They are then rinsed and soaped.

65 A deep greenish black shade is obtained.

(4) PREPARATION OF A MIXED SHADE ON COTTON  
 PIECE GOODS

65 Bleached cotton material is grounded on a  
 foulard at about 50° C. in the following solution:

15 grams of 1-(2',3'-hydroxynaphthoyl)-amino-  
 2-methoxy-benzene are made into a  
 paste with  
 70 15 cc. of Turkey red oil and  
 22.5 cc. of caustic soda solution of 34° Bé. The  
 paste is dissolved in hot water and  
 made up to

75 1 liter.

The impregnated and dried material is then  
 passed at about 20° C. on a foulard through the  
 following solution:

7 grams of the diazonium chloride from 4-  
 amino-4'-methoxy-diphenylamine, 5  
 3.5 grams of the diazonium chloride from 4-  
 amino-3,4'-dinitro-diphenylamine and  
 10 10 grams of ammonium sulfate are dissolved in  
 water and made up to 10

1 liter.

The material is passed through the solution and  
 then through a steam chest in which it is steamed  
 for about half a minute. Then it is rinsed and  
 soaped. 15

A reddish blue-black shade is obtained.

(5) 11.8 grams of 3,4'-dinitrodiphenylamine-4-  
 diazonium chloride of net content 20  
 of 59 per cent are dissolved in  
 300 cc. of decinormal acetic acid and  
 1500 cc. of water.

The following solution is then added, while stir-  
 ring: 25

10.6 grams of 2,3-hydroxynaphthoyl-amino-  
 benzene,  
 200 cc. of decinormal caustic soda solu-  
 tion in  
 1000 cc. of water. 30

The black dyestuff so obtained is filtered with  
 suction and washed well. For the production of  
 pigments it is advantageously used in the form of  
 a paste. 35

Since an object of the present invention is to  
 provide dyestuffs of good fastness properties  
 which dyestuffs are insoluble in water and al-  
 kalies, it is to be understood that the aromatic  
 nuclei of the general formulae appearing in the  
 appended claims do not contain any substituents  
 40 which are known to render organic compounds  
 soluble in water or alkalies and to tend to depre-  
 ciate the fastness of the dyestuffs to alkalies.  
 Substituents of this kind are, for instance, the  
 sulfonic acid and the carboxylic acid group. 45

We claim:

1. The water-insoluble azo-dyestuffs of the fol-  
 lowing general formula: 50



wherein X stands for hydrogen, bromine or  
 60 methoxy and R for a radical of the benzene or  
 naphthalene series, yielding, when produced on  
 the fiber, black-currant to black dyeings of good  
 fastness properties, particularly of very good  
 fastness to light.

2. The water-insoluble azo-dyestuffs of the fol-  
 lowing general formula: 65



wherein R stands for a radical of the benzene 75

series, yielding, when produced on the fiber, black-currant to black dyeings of good fastness properties, particularly of very good fastness to light.

3. The water-insoluble azo-dyestuff of the following formula:



15 yielding, when produced on the fiber, greenish black dyeings of good fastness properties, particularly of very good fastness to light.

4. The water-insoluble azo-dyestuff of the following formula:



25 yielding, when produced on the fiber, greenish

black dyeings of good fastness properties, particularly of very good fastness to light.

5. The water-insoluble azo-dyestuff of the following formula:



10 yielding, when produced on the fiber, violet-black dyeings of good fastness properties, particularly 15 of very good fastness to light.

6. Fiber dyed with the dyestuffs as claimed in claim 1.

7. Fiber dyed with the dyestuffs as claimed in claim 2.

8. Fiber dyed with the dyestuff as claimed in 20 claim 3.

9. Fiber dyed with the dyestuff as claimed in claim 4.

10. Fiber dyed with the dyestuff as claimed in 25 claim 5.

LEOPOLD LASKA.  
ARTHUR ZITSCHER.  
WILHELM SEIDENFADEN.